

1

3,203,800

PHOTOGRAPHIC MATERIAL COMPRISING A SILVER HALIDE EMULSION CONTAINING AN ANTI-BRONZING AGENT

Jozef Frans Willems, Hendrik Adolf Pattijn, and Gerard Michiel Sevens, Wilrijk-Antwerp, Belgium, assignors to Gevaert Photo-Producten N.V., Mortsel-Antwerp, Belgium, a company of Belgium

No Drawing. Filed Jan. 7, 1963, Ser. No. 249,615  
Claims priority, application Belgium, Jan. 5, 1962,

41,269, Patent 612,311  
4 Claims. (Cl. 96—67)

This invention relates to photographic material which is protected against bronzing caused by hot glazing or mechanical drying.

The images obtained in light-sensitive silver halide emulsion layers often undergo changes during processing among others during hot glazing or mechanical drying, at high temperature. During these treatments loss of density occurs easily by the so-called "bronzing" of the silver image.

It is known to add small amounts of chemical compounds to light-sensitive materials containing silver halide or to certain processing baths in order to avoid decrease of density as a result of high glossing.

In addition to the fact that these compounds do not completely counteract bronzing, they still show other disadvantages when being added to a silver halide emulsion.

The most important disadvantage is their mostly very strong desensitizing action.

It has now been found that by adding compounds according to the following general formula:



wherein:

$R_1$  represents an aryl group or a substituted aryl group,  $R_2$  represents a hydrogen atom, an alkyl group, a substituted alkyl group, an aryl group or a substituted aryl group,

Each of  $R_3$  and  $R_4$  (same or different) represent a hydrogen atom, a lower alkyl group or a substituted lower alkyl group, and

$n$  represents a positive integer from 1 to 5,

to the light-sensitive silver halide emulsion layer and/or to at least one water-permeable layer of the light-sensitive material at the same side of the support as said emulsion layer, the disadvantages caused by hot glazing or mechanical drying are prevented.

Contrary to suchlike compounds with a free mercapto function, these compounds have no desensitizing action on the silver halide emulsion.

Suitable compounds corresponding to the above general formula are e.g.:



silver salt of  $\alpha$ -mercaptopropionic acid-p-toluidide



silver salt of  $\beta$ -mercaptopropionic acid-p-toluidide



silver salt of  $\alpha$ -mercaptopropionic acid-anilide

2



5 silver salt of  $\alpha$ -mercaptopropionic acid-1-naphthalide



10 silver salt of  $\alpha$ -mercaptopropionic acid-2-naphthalide



15 silver salt of N-phenyl- $\alpha$ -mercaptopropionic acid-anilide



20 silver salt of  $\alpha$ -mercaptopropionic acid-p-toluidide



25 silver salt of  $\alpha$ -mercaptopropionic acid-p-toluidide

30 The light-sensitive silver halide emulsion wherein compounds according to the present invention can be incorporated can be any silver halide emulsion such as a gelatino-silver chloride emulsion, a gelatino-silver chloro-bromide emulsion, a gelatino-silver chloroiodide emulsion, a gelatino-silver bromide emulsion, a gelatino-silver bromoiodide emulsion, and a gelatino-silver chlorobromoiodide emulsion. The emulsion can be sensitized chemically as well as optically. It may moreover contain all known additives such as anti-fogging agents, stabilizers, hardening agents, softening agents and dispersing agents.

35 The compounds according to the present invention can be added during any stage of the preparation of the emulsion, e.g. during the formation of the silver halide or during the physical or chemical ripening, but preferably after the chemical ripening.

40 The amount, in which the compounds according to the present invention may be added depends on the emulsion used but it generally varies from 2 to 20 g. per 1000 g. of silver nitrate.

45 The compounds according to the present invention are present in the light-sensitive composition in the form of a colloidal dispersion.

50 When using the compounds according to the present invention, there is no loss in sensitivity or contrast of the photographic material, whereas the use of the compounds in their free mercapto form or as alkaline metal or ammonium salt would cause a considerable loss in sensitivity.

55 It is also possible to incorporate the compounds according to the present invention in a hydrophilic layer adjacent to the light-sensitive layer e.g. in the covering layer, or in another layer from which, during fixation, they can e.g. diffuse to the silver halide emulsion layer. The concentration in which the compounds according to the invention are incorporated into these layers is mostly the same as or slightly higher than their concentration when added to the light-sensitive layer.

60 The compounds according to the invention are sometimes incorporated into a processing bath e.g. in the fixing bath.

65 The combination of at least one of the compounds

according to this invention with poly(N-vinylpyrrolidone) gives as anti-bronzing agent still better results. In that case poly(N-vinylpyrrolidone) can be incorporated into the light-sensitive layer and/or into an other water-permeable layer at the same side of the support as the light-sensitive layer, in a concentration which preferably varies from 20 to 80 g. per mole of silver halide.

The following are examples illustrating the properties of photographic materials containing anti-bronzing agents according to the present invention.

*Example 1*

To an ammoniacal gelatino-silver bromoiodide emulsion containing 3.5 mol percent of silver iodide based on the total amount of silver halide and having a medium gradation are added per mole of silver halide 1.9 g. of the silver salt of  $\alpha$ -mercapto-butyric acid-p-toluidide in the form of a dispersion. This emulsion is applied on a baryta-coated paper support in such a way, the light-sensitive layer contains per sq. m. an amount of silver halide equivalent to 2 g. of silver nitrate. On this emulsion layer a gelatin-containing covering layer is coated. This material is exposed under a step-wedge, developed, fixed and rinsed. Then it is subjected to high glossing by pressing its image side against a heated polished metal surface. The reflection densities are measured by means of a MacBeth densitometer before and after subjecting the material to high glossing. The following results are obtained:

|                                                                                     | Maximum density                            |                                           |
|-------------------------------------------------------------------------------------|--------------------------------------------|-------------------------------------------|
|                                                                                     | Before sub-<br>jecting to<br>high glossing | After sub-<br>jecting to<br>high glossing |
| Comparison material (comprising no anti-bronzing agent according to this invention) | 2.09                                       | 1.84                                      |
| Material as described above, comprising the above mentioned anti-bronzing agent     | 2.10                                       | 2.00                                      |

*Example 2*

Three materials are prepared starting from an ammoniacal gelatino-silver bromoiodide emulsion as described in Example 1. In the preparation of the first material (the comparison material), no anti-bronzing agent is added to the emulsion. In the preparation of the second and the third material, respectively of 0.45 g. of the silver salt of  $\alpha$ -mercapto-butyric acid-p-toluidide and 0.45 g. of the silver salt of  $\beta$ -mercapto-propionic acid-p-toluidide are added to the emulsion per mol of silver halide. Moreover, in the preparation of the three emulsions, 60 g. of poly(N-vinylpyrrolidone) are added per mol of silver halide. The emulsions are applied to baryta-coated paper supports in such a way, that the light-sensitive layer contains per sq. m. an amount of silver

halide equivalent to 2.2 g. of silver nitrate. On the emulsion layers gelatin-containing covering layers are coated. The three materials thus obtained are then treated in the same way as in Example 1. The results are the following.

| 10                                   | Maximum density                            |                                           |
|--------------------------------------|--------------------------------------------|-------------------------------------------|
|                                      | Before sub-<br>jecting to<br>high glossing | After sub-<br>jecting to<br>high glossing |
| First material (comparison material) | 2.04                                       | 1.93                                      |
| Second material                      | 2.10                                       | 2.06                                      |
| Third material                       | 2.11                                       | 2.02                                      |

15 From these two examples it appears that poly(N-vinylpyrrolidone) has also a certain anti-bronzing action.

We claim:

20 1. A photographic material comprising a support and at least one light-sensitive silver-halide emulsion layer and containing the silver salt of a member of the group consisting of  $\alpha$ -mercapto butyric acid-p-toluidide,  $\beta$ -mercapto-propionic acid-p-toluidide,  $\alpha$ -mercapto-acetanilide,  $\alpha$ -mercaptobutyric acid-1-naphthalide,  $\alpha$ -mercapto-acetic acid-2-naphthalide, N-phenyl- $\alpha$ -mercapto-butyric acid-anilide,  $\alpha$ -mercapto-propionic acid-p-toluidide, and  $\alpha$ -mercapto-isobutyric acid-p-toluidide in at least one water-permeable layer which is situated at the same side of the support as the light-sensitive silver-halide emulsion layer.

25 2. A photographic material comprising a support and at least one light-sensitive silver halide emulsion layer and containing the silver salt of  $\beta$ -mercapto-propionic acid-p-toluidide in at least one water-permeable layer which is situated at the same side of the support as the light-sensitive silver halide emulsion layer.

30 3. A photographic material comprising a support and at least one light-sensitive silver halide emulsion layer and containing the silver salt of  $\beta$ -mercapto-propionic acid-p-toluidide in at least one water-permeable layer which is situated at the same side of the support as the light-sensitive silver halide emulsion layer.

35 4. The photographic material of claim 1 wherein the water-permeable layer contains poly(N-vinylpyrrolidone).

**References Cited by the Examiner**

**UNITED STATES PATENTS**

3,080,230 3/63 Haydn et al. ----- 96—95

**FOREIGN PATENTS**

1,090,385 3/55 France.

794,637 5/58 Great Britain.

607,639 10/60 Canada.

55 1,119,119 12/61 Germany.

NORMAN G. TORCHIN, Primary Examiner.